

# UNITED STATES PATENT OFFICE.

JOHN E. SAWYER, OF NAPA, CALIFORNIA.

## LUBRICATING COMPOUND.

SPECIFICATION forming part of Letters Patent No. 268,546, dated December 5, 1882.  
Application filed July 25, 1882. (No specimens.)

*To all whom it may concern:*

Be it known that I, JOHN E. SAWYER, a citizen of the United States, residing at Napa, in the county of Napa and State of California, have invented a new and useful Composition of Matter for Lubricating Purposes, of which the following is a specification.

My composition consists of the following ingredients, combined in the following proportions stated, to wit: tallow, sixteen (16) pounds; plumbago or black-lead, one (1) pound; fuller's-earth, one-half ( $\frac{1}{2}$ ) pound; soapstone or steatite, one-half ( $\frac{1}{2}$ ) pound; lard-oil, one (1) pint. The soapstone, plumbago, and fuller's-earth are pulverized and the tallow melted, when the soapstone, plumbago, fuller's-earth, and lard-oil are mixed with the tallow, and the whole passed through a grinding-mill and thoroughly mixed and incorporated by grinding while the tallow is in a hot or melted state. By this means the composition will always remain in a limpid or plastic state, and will not cake or harden in the containing-can, and when applied to axles will remain a

long time without a new application; and it will also prevent the heating of the axle to which it is applied.

I am aware that steatite or soapstone and black-lead or plumbago have heretofore been employed in lubricating compounds; but I am not aware that all of the ingredients of my compound, in the proportions stated, have been used together.

Having thus described my invention, what I claim, and desire to secure by Letters Patent, is—

The herein-described composition to be used as a lubricant, consisting of tallow, plumbago, soapstone, fuller's-earth, and lard-oil, mixed and compounded in the proportions stated.

In testimony that I claim the foregoing I have hereunto set my hand and seal this 26th day of June, 1882.

J. E. SAWYER. [L. S.]

Witnesses:

CHAS. E. KELLY,  
WILMER BRADFORD.